

April 11, 1939.

G. J. EASTER ET AL

2,154,153

REFRACTORY AND METHOD OF MAKING IT

Filed July 21, 1936

*Fig. 1.*



*Fig. 2.*



BY

INVENTOR.  
GEORGE J. EASTER  
KARL BROWNELL

*R.C. Benner*

ATTORNEY.

## UNITED STATES PATENT OFFICE

2,154,153

## REFRACTORY AND METHOD OF MAKING IT

George J. Easter and Karl Brownell, Niagara Falls, N. Y., assignors, by mesne assignments, to The Carborundum Company, Niagara Falls, N. Y., a corporation of Delaware

Application July 21, 1936, Serial No. 91,748

10 Claims. (Cl. 49—79)

This invention relates to an improvement in refractory articles and the method of making them, and particularly to refractory articles which are cast in monolithic form from a molten mass.

In the manufacture of cast refractories which are made by pouring molten material into a mold, serious difficulty is encountered in securing castings which are solid throughout and which are not characterized by a pipe or hollow in the center of the casting. This is particularly true in the case of castings composed of 85% or more of alumina, because material of that type shows a volume shrinkage of approximately 20% as it cools down from the molten condition to the point at which it solidifies. Certain mixtures, notably beta alumina, do not show this shrinkage and accordingly do not tend to have hollows in the center of the casting. Our invention is, however, advantageous in certain respects for use with castings of even this latter material. This is because the object of this invention is not merely to produce solid castings, but also to accelerate the solidification of the casting and to provide an interlocking internal structure which increases the strength of the casting and moreover permits profitable utilization of a considerable quantity of material which would otherwise be wasted.

In the previous work on the casting of refractories, the tendency toward piping has been constantly objectionable and efforts have been made to overcome the difficulty in various ways, as, for instance by providing a casting with a very large font or header from which the still molten material could drain down into the casting proper as the latter solidified. This has been successful only in instances where the font has been of inordinately large size and has resulted in the loss of excessive quantity of material when the header was scrapped. Attempts have also been made to secure solid castings by multiple pouring, whereby the casting is allowed to cool and shrink and the font is then refilled with additional molten material which is supposed to run in and take the place of the material which previously occupied the cavity in the center of the block. This has been only partially successful, inasmuch as great care is necessary to pour the second charge at exactly the right time. If it is poured too late the secondary material fails to knit together with the former supply and results in a physically weak casting. Moreover, it is frequently found that the gate leading from the font to the casting proper freezes up so solidly

that the secondary charge cannot penetrate into the cavity in the block.

By our method, these disadvantages are overcome and we secure a cast block which has no central cavity but is instead solid throughout and possesses a structure which greatly increases its strength and decreases its tendency to crack during the process of manufacture. The time required for manipulation of the casting during the filling of the central cavity is, moreover, decreased from around 40 minutes to perhaps 10 minutes.

Our method is briefly to cast the molten material in the usual manner and thereafter use an electric arc to keep the font full of molten material and the gate open while we add to the center of the casting lumps of material such, for instance, as pieces of scrap formed from the broken headers from previous castings, thereby chilling the center of the casting so as to cause it to solidify at approximately the same time as the outer portions. In this way, relatively small fonts or headers are sufficient and the material which forms them is, to a considerable extent, ultimately salvaged and fed into the center of succeeding castings. While this reuse of scrap is advantageous, our invention is not limited to the use of such material but contemplates the addition of any relatively cold solid material in the manner indicated.

In the accompanying drawing,

Fig. 1 shows a section through the center of a casting in a mold immediately at the conclusion of the casting operation; and

Fig. 2 shows a section through the center of a casting near the conclusion of our subsequent treatment.

We shall now explain our method of procedure by describing the manufacture of a casting made of fused alumina, such for example as the fused alumina secured as excess fines from the abrasive industry. This material is composed of approximately 95% alumina, the remainder being miscellaneous impurities such as titania, silica, iron oxide, etc. This example is chosen at random as one of numerous materials to which we have found our invention applicable and is to be regarded as an example rather than as a limiting disclosure.

In the manufacture of cast refractories, we first prepare a melt in an electric arc furnace in the manner well known to operators in the abrasive industry and as described in several patents relating to cast refractories. When the material has become molten and its chemical and

physical characteristics have been adjusted to the desired condition in the usual way, we pour the molten material into a mold, which in Fig. 1 is designated as 1. This mold may be made of 5 cast iron, graphite slabs or granular refractory material. It should, however, preferably be made of slabs which are clamped together and can be quickly disassembled when so desired. The mold is surmounted by a cover 2 preferably 10 of graphite slabs, having a center opening or gate which is preferably tapered as illustrated in the drawing. This cover is held in place by a heavy font-retaining ring 3 which surrounds the gate.

15 The molten material 4 is poured into the mold up to the top of the retaining ring 3, and the casting allowed to stand for a few minutes while solidification occurs next to the mold walls. As soon as these walls form sufficiently to be self- 20 supporting, the mold sides are removed and a sheet iron ring 5 placed around the casting several inches away from it. This intervening space is then filled with insulating material 6 such as finely divided alumina or "Sil-O-Cel". Any crust 25 which has formed over the header is now broken and, if need be, more molten material added to again bring the level of molten material up to a point where it can be contacted by electrodes 7, which are connected to a source of electric current 30 (not shown) and are suspended in such a manner that their position is readily adjustable. These electrodes are lowered into the melt in the font and a current passed between them. If necessary this current may be started by using a 35 small carbon rod to make contact between the electrodes.

Alternatively, instead of allowing the casting to stand for a few minutes before the electrodes are inserted, they may be inserted in the font immediately after casting and additional charge 40 melted in the font to supply the requirements as shrinkage draws molten material into the casting below.

As soon as is practical after the casting has first been poured, we have found it advantageous to remove the slabs which form the mold walls. In this way, damage to the mold itself is minimized and the tendency of the casting to crack upon cooling is considerably decreased.

5 The presence of the arc in the header maintains the alumina or other cast material in the header and upper portion of the casting at a high degree of fluidity and prevents premature closing of the gate between the header and casting. Additional fused material may be added from an outside source or unfused material may be fed into this miniature arc furnace at this stage so that it becomes molten and flows down into the center of the casting, replacing material which tends to contract as the casting solidifies.

As soon as the molten material has solidified for a short distance inward from the mold faces, as perhaps to the position indicated by a dotted line 8, we drop into the molten font irregular lumps 9 of cold material of any convenient shape. These lumps may be made from the headers from previous castings or from any other source. While in general we prefer that they should be of the same composition as the casting itself, it is permissible to use lumps of other high refractory materials which do not react chemically with the melt which is being cast. These lumps 9 which are in general cold and hence of greater density than the molten material, tend to sink promptly through the molten material until they

come to rest in contact with the outer solidified shell of the casting. We prefer to add these lumps at regular intervals, a few seconds apart, for example at the rate of one lump approximately every eight (8) seconds in making castings approximately one foot cube. In this way the lumps become sufficiently heated on their outsides by contact with the molten bath to become integrally welded into the structure of the block. The lumps may be conveniently dropped through 10 a funnel mouthed pipe (not shown) terminating six or eight (6 or 8) inches above the bath. This drops them into the bath at the proper point and protects the operator from the heat.

15 It is usually possible to locate the approximate boundary of such lumps in a broken casting, but in general we prefer that the lumps should be so proportioned and so slowly added that there is no separating crack at the interface between the lump and the surrounding matrix material. 20 The size of lumps which can be added varies somewhat in proportion to the dimensions of the casting, pieces approximately 1 inch across being desirable for light castings such as 9 x 10 x 12 inches, whereas on 18 inch castings, 2 inch lumps 25 are permissible and on larger pieces even larger lumps may be used.

This gradual addition of lump material is continued until it is ascertained by poking into the melt with an iron or carbon rod that the material in the casting proper is no longer fluid. When this stage is reached one or two more lumps are added and the electrodes are then withdrawn, the mold cover 2 and retaining ring 3 removed, and the block covered with finely divided alumina or other insulating material and allowed to cool slowly or it may be placed in a furnace and brought down to room temperature sufficiently slowly to prevent cracking.

30 Addition of lumps in this way permits them to become firmly welded into the structure of the casting as a whole, each being substantially surrounded by a subsequently solidified matrix which in general prevents their direct contact with one another. A considerable volume of material may 45 be added in this way, amounting to from 15 to 30% of the weight of the entire casting. The added lumps act as a sort of tie-rod, binding the refractory together so that its strength in service is materially superior to the strength of similar pieces to which lumps have not been added.

50 The porosity of the casing is not materially affected except that the central cavity is eliminated. We have, for instance, made castings with as low as 3% porosity by this method. Where the material is intentionally made porous, the porosity is not materially reduced except insofar as the added chunks may be of more solid stock.

55 We have had successful results not only by adding alpha alumina chunks to alpha and beta alumina castings, but also to mullite castings and vice versa. In general, it is preferable that the lumps added be of the same material as the surrounding matrix except in isolated instances where the solid material is less dense than the molten form so that the lumps float on top instead of sinking into the casting proper. This condition prevails, for instance, with beta alumina where the solid material seems to be less dense 65 than the melt from which it forms.

70 Due to the fact that the interior of the casting transfers its heat to the cold lumps, the temperature of the interior portion falls off rapidly to the solidification point while the temperature

of the outer portion of the casting remains almost as high. This results in a very material decrease in the strains which are otherwise set up due to shrinkage resulting from the more 5 rapid cooling of the outer shell and delayed solidification of the center of the casting. This result is quite beneficial throughout the entire life of the block and considerably simplifies the annealing practice. The presence of the added 10 lumps does not affect the general character of the crystalline structure of the casting, but rather permits it to be either coarsely crystalline with strongly oriented crystals or finely crystalline without predominant orientation, depending upon 15 the other conditions of casting, such, for instance, as the temperature of pouring.

By utilizing our process as above described, we produce a new and valuable block structure in the case of materials having strong crystallizing proclivities (such as alumina or mullite) when the original casting is poured when the melt is well above its fusion point. Blocks made in this way to which lumps are then added show an outer shell of coarsely crystalline, highly 20 oriented material, which (as described in pending application Serial #51,113 filed November 22, 1935, by Easter and Benner) is very beneficial for use in resisting slag attack. Inside this outer shell, however, the crystals, while relatively coarse, are found to be oriented in clusters 25 in which they radiate out for an inch or more from the inserted lumps. This structure is illustrated diagrammatically in Fig. 2. It produces a block which combines the advantages of high 30 mechanical strength with the superior slag resisting qualities associated with oriented crystals.

This structure is not secured when the melt is allowed to closely approach its solidification point before pouring. In either case the major 40 portion of the block retains its characteristic crystal orientation and the structure of only the innermost 15 to 40% of it is in any way affected by the added lumps. In either case the block is strong, solid and very serviceable as a refractory.

Having thus described our invention and recited by way of illustration its application to the formation of a casting of fused alumina, we wish to secure protection for our invention within the scope of the following claims.

50 We claim:

1. The method of forming refractory castings which comprises casting molten refractory material into a mold having a superimposed font separated therefrom by a gate and after solidification of a layer of refractory material about the inner walls of said mold, maintaining the material in the interior of the font and gate fluid by means of an electric arc and feeding lumps of solid refractory material through said fluid 55 into the interior of the casting, thereby accelerating and causing the solidification of the interior of the casting before complete melting of the added lumps.

2. The method of fabricating castings of refractory materials which comprises supplying 60

molten refractory material to a mold to form a casting and adding lumps of solid refractory material into the interior of the casting to hasten solidification thereof said solidification taking place before complete liquidation of the added lumps but after said lumps have started to melt while keeping the upper surface of the casting fluid.

3. In the process of manufacturing fused cast refractories, the steps which comprise supplying 1 molten refractory material to a mold to form a casting and adding lumps of relatively cold refractory material to the interior of the casting after the walls thereof have congealed to solidify the interior after incipient fusion of the added lumps but before said lumps have lost their identity.

4. A casting composed of refractory oxides and having in the interior portion only thereof coarse lumps of refractory oxide, said lumps being substantially surrounded by a subsequently solidified matrix.

5. A refractory casting comprising in the interior portion thereof previously solidified lumps integrally fused into the structure of the casting, and adjacent its outer edges a layer free 25 from such lumps.

6. A refractory casting comprising in the interior portion only thereof previously solidified lumps, which lumps are integrally fused into the structure of the casting yet retain their identity.

7. In a refractory casting composed of crystalline oxidic material, an outer shell of distinctly oriented crystals and within said shell a zone characterized by differently oriented crystals surrounding lumps of refractory material having still different orientation of the crystals composing them.

8. The process of making refractory castings which comprises supplying molten refractory material to a mold, allowing said molten material to congeal adjacent the mold whereby a characteristic orientation of the crystals in the said congealed portion results, and thereafter adding to the interior of the casting cold refractory material to accelerate solidification thereof said interior solidifying after incipient melting of the added cold material but before said material loses its identity.

9. A refractory casting consisting of at least 50 85% aluminum, in which casting the interior only comprises irregular pieces of refractory material distinct from but integrally fused together with their surrounding matrix.

10. A casting composed of oxidic refractory material and consisting of a shell of solidified molten material enclosing in the central portion only thereof a subsequently solidified matrix and irregularly distributed, substantially separated lumps of previously solidified molten refractory material, said lumps and matrix being integrally fused together.

GEORGE J. EASTER.  
KARL BROWNELL.

CERTIFICATE OF CORRECTION.

Patent No. 2,154,153.

April 11, 1939.

GEORGE J. EASTER, ET AL.

It is hereby certified that error appears in the printed specification of the above numbered patent requiring correction as follows: Page 3, second column, line 51, claim 9, for "aluminum" read alumina; and that the said Letters Patent should be read with this correction therein that the same may conform to the record of the case in the Patent Office.

Signed and sealed this 27th day of June, A. D. 1939.

(Seal)

Henry Van Arsdale  
Acting Commissioner of Patents.